

## UNITED STATES PATENT OFFICE

2,480,753

METHOD OF PRODUCING AN ADSORBENT  
CLEANING MATERIAL

William S. W. McCarter, Bala-Cynwyd, Pa., assignor to Attapulgus Clay Company, Philadelphia, Pa., a corporation of Delaware

No Drawing. Application November 28, 1945,  
Serial No. 631,479

4 Claims. (Cl. 252—89)

1

The present invention relates to improved adsorbent cleaning compositions and method of making same, and relates more particularly to low density, highly adsorptive clay-type compositions suitable for use in removing oil, grease, water and the like from surfaces such as wooden or concrete floors, linoleum, paper and fabrics.

I have found that satisfactory cleaning compositions should be characterized by a high oil retention, a low density or volume weight, and a high resistance to attrition or breakdown upon use. Low bulk density or volume weight is desired because the lower the volume weight, the greater the surface area which can be covered by a given weight of cleaning composition. Hardness or resistance to attrition is necessary, since a soft, readily powdered material is difficult to remove from the surface being cleaned. High oil retention is desirable in order that a minimum amount of the cleaning composition may be used in removing oil, grease and the like from the surface being cleaned.

It is obvious, however, that a decrease in volume weight of the cleaning composition without any change in other properties does not constitute an improvement. For example, let it be assumed that two adsorbent cleaners have the same oil retention upon a weight basis, but that the first cleaner has one-half the volume weight of the second. The first cleaner will have twice the covering power of the second, assuming that layers of equal thickness are used. In spite of the greater covering power, the first cleaner is not better than the second because in order to adsorb the same amount of oil per unit area, the layer of the first cleaner would have to be twice as thick as that of the second cleaner. In general, a lowering of volume weight is desirable if the oil retention can be increased correspondingly, and the factor which shows the relative merits of various cleaners is the oil retention on the volume basis.

I have found that improved adsorbent cleaning compositions may be prepared by incorporating with a plastic adsorbent clay, a suitable quantity of a cellulosic material, intimately admixing the clay and cellulosic material, drying the mixture, reducing the dried material to granules of desired size, and calcining the granules at elevated temperature.

In accordance with my invention, an adsorbent clay such as fuller's earth is mixed with a cellulosic material such as sawdust, wood flour, or paper pulp, and the water content of the mixture is adjusted by the addition of water, if necessary,

to a value between 40% and 60% by weight, and preferably between 53% and 56% by weight. The ratio of cellulosic material to fuller's earth may range from 1 part to 30 parts by weight. For example, in a sawdust-fuller's earth mixture, the sawdust may represent from 1% to 30% by weight of the mixture, with preferred amounts ranging from 5% to 25%. In a wood flour-fuller's earth mixture the same proportions may be used, and with a paper pulp-fuller's earth mixture, about 1% to 2% of pulp gives satisfactory results. The mixing may be carried out in a pug mill or other conventional mixer, and the plastic mixture is then delivered to an auger extrusion machine 15 provided with a die plate containing a plurality of holes of suitable diameter, for example,  $\frac{1}{4}$  inch to 1 inch in diameter depending upon the size and output of the extrusion machine. The plastic mixture, in passing through the extruder is thoroughly kneaded and compressed, and is discharged through the die plate orifices in the form of cylindrical pieces of irregular length. The extruded material is then dried at temperatures between 200° F. and 300° F. to remove the bulk of 20 the free moisture, and the dried material is then ground and screened to give granules of desired particle size, for example, 10/60 mesh, 30/60 mesh, etc. The granular material is then calcined by heating in a kiln or clay burner at an elevated 25 temperature preferably between 750° F. and 1200° F. until the volatile matter content is reduced to 10% by weight or lower, for example, 1% to 5% by weight. At 750° F. the cellulosic content of the granules is carbonized and partly consumed by oxidation, whereas at 1200° F. the cellulosic content is almost completely removed by oxidation. In either case there is obtained an adsorbent cleaning composition of lower volume weight and higher oil retention than is produced 30 by a similar treatment of fuller's earth without the added cellulosic material. While it is preferred to use an extrusion machine in conjunction with a pug mill to obtain uniformity and hardness of product, the mixing of the fuller's earth and cellulosic material to form a plastic mixture may be carried out in a pug mill alone, and the mixture may be discharged directly into suitable drying equipment. After drying, the mixture is then ground, screened, and calcined as 35 described hereinbefore.

The adsorbent clay employed in accordance with this invention is preferably fuller's earth of the type mined in Georgia and Florida, although earths from other sources may be used. As mined, 40 the raw fuller's earth usually has a total volatile

matter content (mostly water) of the order of 47% to 49% by weight, and this water content must be taken into account in preparing the fuller's earth-cellulosic material mixtures, all calculations being made upon the basis of dry earth. For example, in 100 parts of a plastic mixture suitable for extrusion, the fuller's earth may comprise 39 parts by weight (dry), the cellulosic material 7 parts by weight, and water 54 parts by weight. The proportions of fuller's earth and cellulosic material may vary considerably, but the water content is preferably maintained between 50 and 60 parts per 100 parts of the total mixture. The cellulosic material is preferably sawdust obtained by the fine sawing of kiln-dried wood of a light species such as redwood, although other sawdusts have been found satisfactory. In general, the mesh size of the sawdust should not exceed the maximum mesh size desired in the granulated adsorbent cleaning composition. For example, if the final product is in the form of 10/60 mesh granules, the sawdust or other cellulosic material should not be coarser than 10 mesh. The finer the particles of cellulosic material, the more readily are they uniformly incorporated with the fuller's earth. Wood flour is especially suitable in this respect, and paper pulp less suitable. My invention may be further illustrated by the following examples, which, however, are not to be construed as limiting the scope thereof.

Cellulosic material was added to raw fuller's earth in various ratios, the water content of the mixtures then being adjusted to about 54% by weight. The mixtures were thoroughly pugged in a conventional pug-mill and then charged to an auger extrusion machine provided with a die plate  $\frac{1}{2}$  inch in thickness and containing a plurality of apertures each  $\frac{1}{8}$  inch in diameter. The mixtures were extruded from the die plate apertures at an elevated pressure above 100 pounds per square inch in the form of relatively hard, cylindrical rods of irregular length. The extruded material was dried at  $220^{\circ}$  F. to a moisture content between 15% and 30% by weight, and the dried material was ground and screened to produce granules of 10/60 mesh. The granular material was then calcined at elevated temperature to give a volatile matter content of not more than about

period of time. A graduated glass cylinder of 100 cc. capacity is filled with the granular material and clamped to a reciprocating platform which is raised and lowered through a distance of  $\frac{1}{16}$  inch by means of a cam rotating at 250 R. P. M. The settling device is operated for exactly 5 minutes, and the cylinder is refilled to the 100 cc. mark by carefully adding more granular material through a funnel, the cylinder not being moved or jarred during the addition of the "make-up." The cylinder and contents is weighed to the nearest 0.1 gram, then emptied and weighed empty. The difference represents the weight of 100 cc. of granular material, which is readily converted to pounds per cubic foot.

Oil retention on a weight basis was obtained by mixing 50 grams of the granular material with an excess of a standard lubricating oil described below, pouring the mixture on a 4 inch Buchner funnel and sucking the contents of the funnel dry by applying reduced pressure (16 inches mercury) for 2 hours at  $150^{\circ}$  F. The granular material is reweighed and the gain in weight is retained oil. From the value found for 50 grams of material, the oil retention in pounds per pound of material can readily be calculated. To determine the oil retention on the volume basis, it is necessary only to multiply the volume weight of the granular material by the value for the oil retention on the weight basis. The oil employed had the following properties:

Saybold universal viscosity at  $100^{\circ}$  F.

seconds 716

Saybolt universal viscosity at  $210^{\circ}$  F.

seconds 624

A. P. I. gravity degrees 21.3

Flash point °F. 405

Fire point °F. 480

Pour test °F. 0

Color (A. S. T. M.) 3½

Other lubricating oils of generally similar properties, particularly viscosity, may be used in lieu of the above without materially changing the test results.

The results of the tests on compositions prepared as hereinbefore described are given in the following table.

|                     | Percent Cellulosic Material Added | Calcined at °F. | Volatile Matter, Percent | Volume Weight, lbs./cu. ft. | Oil Retent. Weight, lbs. per lb. | Oil Retent. Volume, lbs./cu. ft. |
|---------------------|-----------------------------------|-----------------|--------------------------|-----------------------------|----------------------------------|----------------------------------|
| Redwood sawdust     | None                              | 750             | 5.3                      | 34.5                        | 0.716                            | 24.7                             |
|                     | 5                                 | 750             | 4.2                      | 29.9                        | 0.838                            | 25.1                             |
|                     | 15                                | 750             | 4.8                      | 28.4                        | 0.876                            | 24.9                             |
|                     | 25                                | 750             | 5.2                      | 28.0                        | 0.882                            | 24.7                             |
| Yellow pine sawdust | 15                                | 750             | 10.0                     | 30.4                        | 0.816                            | 25.7                             |
|                     | 15                                | 1,000           | 4.3                      | 31.6                        | 0.836                            | 26.4                             |
|                     | 25                                | 1,000           | 5.1                      | 29.8                        | 0.867                            | 25.8                             |
| White pine sawdust  | 10                                | 750             | 8.3                      | 30.9                        | 0.800                            | 24.7                             |
|                     | 15                                | 750             | 4.3                      | 31.0                        | 0.836                            | 25.8                             |
|                     | 25                                | 750             | 10.0                     | 29.7                        | 0.574                            | 25.9                             |
| Paper pulp          | 1.1                               | 750             | 4.4                      | 30.8                        | 0.800                            | 24.1                             |
|                     | 2.6                               | 750             | 4.5                      | 29.1                        | 0.876                            | 26.6                             |

10% by weight. The volatile matter content was determined by heating a weighed sample at  $1800^{\circ}$  F. for 30 minutes, cooling and reweighing to obtain the percent loss. The calcined granular material was tested for volume weight and for oil retention according to the followed methods.

Volume weight was obtained by settling the granular material under regulated conditions. Reproducible settling conditions are achieved through the use of a device which repeatedly lifts and drops a container of the material a fixed distance, at a definite rate, and for a measured

From the above data, it will be seen that improved adsorbent cleaning compositions may be obtained by incorporating finely divided cellulosic material with the fuller's earth, extruding the mixture, and calcining the granular product. In general, I have found that compositions, particularly 10/60 mesh compositions having a volume weight between 26 and 32 pounds per cubic foot, an oil retention between 0.8 and 0.9 pounds per pound of earth, and between 24 and 27 pounds per cubic foot of earth, and a volatile matter content of not more than 10%, are markedly superior to

ordinary fuller's earth as cleaner for oil, grease, and the like. My improvement resides in decreasing the volume weight, thereby increasing the covering power, without adversely affecting the oil retention on the volume basis. In employing a cellulosic material in amounts ranging from 1% to 30%, and preferably from 5% to 25%, I am able to produce highly efficient cleaning compositions having a satisfactory hardness and resistance to disintegration, whereas with more than about 30% of cellulosic material, the product usually is characterized by an undesirable softness.

I claim:

1. A method of producing an adsorbent cleaning material, comprising forming a mixture of from 1 to 30 parts by weight of cellulosic material selected from the group consisting of sawdust, wood flour, and paper pulp, and from 99 to 70 parts by weight of fuller's earth, adjusting the water content of the mixture to a value between 40% and 60% by weight, extruding the mixture at elevated pressure above 100 pounds per square inch, drying the extruded mixture, reducing the dried mixture to granular particles, and calcining the particles at a temperature between 750° F. and 1200° F. for a period of time sufficient to obtain a volatile matter content between 1% and 10% by weight.

2. A method of producing an adsorbent cleaning material, comprising forming a mixture of from 1 to 30 parts by weight of sawdust and from 99 to 70 parts by weight of fuller's earth, adjusting the water content of the mixture to a value between 40% and 60% by weight, extruding the mixture at elevated pressure above 100 pounds per square inch, drying the extruded mixture, reducing the dried mixture to granular particles, and calcining the particles at a temperature between 750° F. and 1200° F. for a period of time sufficient to obtain a volatile matter content between 1% and 10% by weight.

3. A method of producing an adsorbent cleaning material, comprising adding 1 to 30 parts by weight of sawdust and 99 to 70 parts by weight of fuller's earth, adjusting the water content of the mixture to a value between 40% and 60% by weight, thoroughly mixing the sawdust and ful-

ler's earth to obtain a homogeneous dispersion of sawdust in the earth, drying the resulting mixture, reducing the dried mixture to granular particles, and calcining the particles at a temperature between 750° F. and 1200° F. for a period of time sufficient to obtain a volatile matter content between 1% and 10% by weight.

4. An adsorbent cleaning material consisting essentially of granular fuller's earth of 10 to 60 mesh and having a volume weight between 26 and 32 pounds per cubic foot, an oil retention between 0.8 and 0.9 pounds per pound of earth and between 24 and 27 pounds per cubic foot of earth, and a volatile matter content between 1% and 10% by weight, said cleaning material being produced by forming a mixture of from 1 to 30 parts by weight of a cellulosic material selected from the group consisting of sawdust, wood flour, and paper pulp, and from 99 to 70 parts by weight of fuller's earth, adjusting the water content of the mixture to a value between 40% and 60% by weight, extruding the mixture at elevated pressure above 100 lbs./sq. in., drying the extruded mixture, reducing the dried mixture to granular particles, and calcining the particles at a temperature between 750° F. and 1200° F. for a period of time sufficient to obtain a volatile matter content between 1% and 10% by weight,

WILLIAM S. W. McCARTER.

#### REFERENCES CITED

The following references are of record in the file of this patent:

#### UNITED STATES PATENTS

| Number    | Name          | Date          |
|-----------|---------------|---------------|
| 1,749,317 | Chevalier     | Mar. 14, 1930 |
| 2,315,410 | Simons et al. | Mar. 30, 1943 |
| 2,363,876 | La Lande      | Nov. 28, 1944 |

#### FOREIGN PATENTS

| Number  | Country       | Date |
|---------|---------------|------|
| 362,402 | Great Britain | 1930 |

#### OTHER REFERENCES

Modern Soap and Detergent Industry, Martin (1931), vol. 1, section 3, page 23.